

## UNITED STATES PATENT OFFICE.

WILLIAM HOSKINS, OF CHICAGO, ILLINOIS.

## METHOD OF AND COMPOUND FOR REMOVING FROM THE BARRELS OF FIREARMS THE RESIDUES DEPOSITED BY LEAD BULLETS AND SMOKELESS AND SEMISMOKELESS POWDER.

No Drawing.

Application filed January 3, 1921. Serial No. 434,761.

This invention consists in a novel method of and compound for removing from the barrels of firearms the residues left after shooting in the firearms cartridges loaded with lead bullets and smokeless or semi-smokeless powder. The removal of the residues left by black powder cartridges and by smokeless cartridges containing jacketed bullets presents no particular difficulty at the present time. The great difficulty has however, been experienced in the case of weapons, particularly those of small caliber, where the bullets are of lead and the powder is either smokeless or semi-smokeless. In such weapons, the residue is a mixture of grease from the bullet lubricant, a considerable quantity of lead from the bullets, and potassium chloride deposited by the primer. The latter is highly hygroscopic and causes after-corrosion unless removed. The lead is insoluble by ordinary cleansing agents and when mechanically mixed with the grease makes it extremely difficult to clean the surface.

I employ a compound or mixture containing a soft abrasive, hard enough to cut lead but not hard enough to cut steel. My preferred compound contains tri-calcium-phosphate. With this I incorporate an emulsifying agent, such as liquid soap, which will emulsify and break up the grease, and water to dissolve the potassium chloride. In the use of this compound the barrel is scrubbed with one or two patches smeared with the mixture of soap, water and a soft abrasive, and is then scrubbed with a series of patches wet with water, or, in the alternative, water may be either run thru the barrel or pumped in and out of the barrel,

using a cleaning-rod after the manner of a syringe. The barrel is finally dried and covered with a moisture-excluding film of oil and grease, in which condition it is perfectly safe from after corrosion.

I preferably mix the aqueous solution of soap and tri-calcium-phosphate to the consistency of cream, because the abrasive has a tendency to settle out and in that condition can readily be shaken up into the mixture before using. Such a cream may suitably be prepared by mixing 18 grams of tri-calcium-phosphate with 100 ccs. of an aqueous solution containing 10% of potash soap. It must be understood, however, that this example is given by way of illustration only and is not intended to be limitative since excellent results are obtained with compositions of widely differing proportions of components.

## I claim:

1. The herein described compound for removing from barrels of firearms the residue from lead bullets and smokeless or semi-smokeless powder comprising water, an emulsifying agent, and an abrasive of the hardness of tri-calcium-phosphate.

2. The herein described method of removing from the barrels of firearms the residue from lead bullets and smokeless or semi-smokeless powder, which consists in simultaneously subjecting the residue to the action of an abrasive hard enough to cut lead and not sufficiently hard to materially cut the steel of the barrel, water, and an emulsifying agent, and subsequently washing and drying the barrel.

WILLIAM HOSKINS.